

G. W. ELMEN.

MAGNET CORE.

APPLICATION FILED APR. 6, 1916. RENEWED JUNE 27, 1918.

1,286,965.

Patented Dec. 10, 1918.

Fig. 1.



Fig. 2.



Inventor:  
Gustaf W. Elmen.  
by L. C. Munro, Atty.

# UNITED STATES PATENT OFFICE.

GUSTAF W. ELMEN, OF BOGOTA, NEW JERSEY, ASSIGNOR TO WESTERN ELECTRIC COMPANY, INCORPORATED, OF NEW YORK, N. Y., A CORPORATION OF NEW YORK.

## MAGNET-CORE.

1,286,965.

Specification of Letters Patent. Patented Dec. 10, 1918.

Application filed April 6, 1916, Serial No. 89,467. Renewed June 27, 1918. Serial No. 242,313.

To all whom it may concern:

Be it known that I, GUSTAF W. ELMEN, originally a subject of the King of Sweden, who arrived in Philadelphia from Sweden 5 on August 1, 1893, when sixteen years of age, declared my intention of becoming a citizen of the United States on October 5, 1900, and again on April 30, 1915, have been a constant resident of the United States 10 since my arrival, but have not taken out my final naturalization papers, am now residing at Bogota, in the county of Bergen and State of New Jersey, and have invented certain new and useful Improvements in Magnet-Cores, of which the following is a full, clear, concise, and exact description.

This invention relates to magnet cores generally, and is particularly useful in connection with cores for loading coils for telephone circuits. Its general object is to provide a new and improved core material which is cheap to manufacture, which is easily formed to the desired shapes, and which possesses to a high degree those characteristics most advantageous in cores for loading coils and other electrical apparatus.

The present invention may be considered an improvement upon the magnet core and process of manufacture described and 30 claimed in an application for Letters Patent in the name of James Buckner Speed, Serial No. 89,409, filed April 6, 1916, for improvements in magnet cores, assigned to the same assignee as the present application. 35 In the preferred embodiment of the Speed invention, as described in the application above mentioned, the core is composed of finely divided iron in the form of "iron by hydrogen" and insulating material, preferably a coating of red iron oxid, separating the particles of iron, said compound being compressed by pressure sufficient to give it a specific gravity approximating that of the iron employed. While iron particles in the 40 form of "iron by hydrogen" are soft and are therefore suitable for core making, the comparatively high cost of this form of iron, and the difficulties of obtaining it without black iron oxid which is objectionable because it is magnetic and is not an insulating 45 material, renders it unsatisfactory as a raw material for the manufacture of cores. It is, however, impossible to obtain satisfactory soft iron particles by grinding up cast 50 or other forms of soft iron, owing to the

fact that such iron does not fracture into small firm particles of the size desired, but becomes a soft, mushy powder. Nor is it possible to obtain satisfactory iron particles by grinding to the desired size hard iron 60 such as the various forms of steel, because particles so obtained cannot be softened by annealing.

The present invention is the result of the discovery that iron obtained by electrolysis 65 can readily be ground into particles of a size suitable for core making, and that said particles can be easily softened by annealing. The present invention, therefore, consists of a magnet core and method of making the same, characterized by the fact that electrolytic iron is employed, and the further fact that the particles of such iron are annealed before they are compressed to 70 form a core.

In the drawing, Figure 1 is a perspective view of a section of a loading coil core made in accordance with the present invention, and Fig. 2 shows a plurality of these sections assembled to form a complete core. It 80 will be understood, however, that this is merely illustrative, and that the invention is not limited to the production of this form of core, but is adapted for the making of 85 cores of many forms, some of which cannot be made economically and satisfactorily of solid iron, plates or wires.

In the making of loading coil cores, the present invention is preferably carried out in the following manner: Electrolytic iron obtained in any well-known manner, (for example, from a cell containing a bath of ferrous ammonium sulfate), after being broken into small pieces is reduced to small particles by grinding in a ball mill. Experience has shown that for the best results, the particles used in core-making should not be larger in size than what will pass through what is known as eighty-mesh screen. Iron particles of this size are heated in any suitable form of furnace to anneal them and to drive off any occluded gases, principally hydrogen, and are then covered with a surface coating of insulating material, preferably red iron oxid. One method of oxidizing the particles which has been found satisfactory is to add to a mass of iron particles approximately 10% by weight of water, and then to heat and stir the mass in the presence of air until dry. The iron parti- 100 105 110

cles which have been obtained, annealed and covered with a surface coating of red iron oxid in the manner just described, are then ready for compression either into bulk material from which cores may be made, or directly into the desired form of core.

The remainder of the method of making magnet cores is substantially the same as that described in the Speed application for patent above referred to; but in order that this application may contain a full disclosure of the best method of carrying out the present invention, the remaining steps of the method will be herein described.

15 The mold and press employed in the compressing process should be capable of standing and exerting exceedingly high pressures. Preferably, pressures as high as two hundred thousand pounds to the square inch should be employed; and for the best results as to uniform density, the thickness of any core section, in the direction in which the pressure is exerted in forming it, should normally not exceed approximately 25 one-quarter of an inch. This consideration is so important that it has been found desirable in making loading coil cores to use core sections even as thin as one-tenth of an inch, and to employ from twelve to fifteen 30 sections in building up a core, a suitable insulating material such as paper, lacquer or shellac being interposed between the sections. Fig. 1 shows such a core section or ring; and Fig. 2 shows the built-up 35 core.

It has been found that cores made in the manner above described are strong mechanically and stable chemically; and that their specific gravity is approximately 40 7, which is nearly that of undivided iron, which is approximately 7, 7. Electrically, a loading coil core of this kind has high specific resistance, an extremely low hysteresis characteristic, excellent magnetic stability, and comparatively high permeability, as understood in telephone loading coil design. The volume permeability of a core increases much more rapidly with increase 45 of specific gravity, the more nearly the specific gravity of the core approaches that of undivided iron. In other words, increases of pressure are increasingly beneficial as far as volume permeability is concerned, even though the intrinsic permeability of the particles has been lowered 55 by reason of their compression. It has been found, however, that the tendency of the oxid coating on the particles to puncture and thereby reduce the resistance of the 60 core section, makes it unwise to use pressures above a certain maximum value. This value depends, of course, upon the char-

acter of the oxid coating on the particles, and in experiments which led to the present invention has been found to be approximately 200,000 pounds per square inch.

What is claimed is:

1. A magnet core composed of finely divided electrolytic iron, and insulating material separating the particles of the iron, 70 said compound being compressed by pressure sufficient to give it a specific gravity approximately the same as that of undivided iron.

2. A magnet core composed of finely 75 divided electrolytic iron, and insulating material separating the particles of the iron, said compound being compressed by pressure sufficient to give it a specific gravity of approximately 80 7.

3. A magnet core composed of finely divided annealed electrolytic iron, and insulating material separating the particles of the iron, said compound being compressed by pressure sufficient to give it a 85 specific gravity approximately the same as that of undivided iron.

4. The method of making magnet cores which consists in reducing electrolytic iron to a finely divided form, annealing the iron 90 particles, coating said particles with insulating material, and submitting a mass of said particles to pressure sufficient to give the mass a specific gravity of approximately 95 7.

5. The method of making magnet cores which consists in reducing electrolytic iron to a finely divided form, annealing the iron particles, coating the surface of said particles with red iron oxid, and submitting a 100 mass of said particles to pressure sufficient to form the mass to the desired shape and to give it a specific gravity of approximately 7.

6. The method of making magnet cores 105 which consists in producing iron electrolytically, grinding said iron into a finely divided state, coating the iron particles with insulating material, and submitting a mass of said particles to pressure sufficient to 110 compress the mass into a self-sustaining solid.

7. The method of making a magnet core which consists in producing iron electrolytically, grinding said iron into a finely 115 divided state, annealing the iron particles, coating said particles with insulating material, and submitting a mass of said particles to pressure sufficient to compress the mass into a self-sustaining solid.

In witness whereof, I hereunto subscribe my name this 4th day of April, A. D., 1916.

GUSTAF W. ELMEN.